# EUROPEAN PATENT SPECIFICATION

(11) **EP 2 113 636 B1**
(45) Date of publication and mention of the grant of the patent: **03.12.2014**
(21) Application number: 09250906.6
(22) Date of filing: 27.03.2009
(51) Int. Cl.: F01D 5/28, F01D 9/04

(54) **Coated turbine-stage nozzle segments**
Beschichtete Turbinstufendüsensegmente
Segments revêtus de distributeur d'étage de turbine

(30) Priority: 02.05.2008 US 151102
(43) Date of publication of application: 04.11.2009
(73) Proprietor: United Technologies Corporation, Hartford, CT 06101 (US)
(72) Inventor: Minor, Michael J., Arlington, TX 76018 (US); Miller, Michael L., Euless, TX 76039 (US); Pellet, Paul M., Arlington, TX 76006 (US)
(74) Representative: Tomlinson, Kerry John

(56) References cited:
- EP-A1- 0 744 529
- EP-A1- 1 544 414
- EP-A1- 1 790 825
- EP-A2- 1 803 896

## Description

### BACKGROUND

The present invention relates to the manufacture and restoration of aerospace components, such as components of gas turbine engines. In particular, the present invention relates to methods for forming coatings on turbine-stage nozzle segments.

Gas turbine engines operate by burning a combustible fuel-air mixture, and converting the energy of combustion into a propulsive force. A gas turbine engine typically includes an inlet, a compressor, a combustor, a turbine, and an exhaust duct, where the compressor draws in ambient air and increases its temperature and pressure. Fuel is added to the compressed air in the combustor, where it is burned to raise the gas temperature, thereby imparting energy to the gas stream. The resulting combustion gases are directed axially rearward from the combustor through an annular duct, where the gases interact with multiple turbine stages disposed within the annular duct.

Each turbine stage includes a stationary turbine nozzle derived of multiple stator vanes, and a downstream row of rotatable blades. The stator vanes direct the combustion gases axially rearward in a downstream direction, and the rotatable blades direct the energy of the combustion gases to an axial drive shaft that is interconnected with the compressor. Stator vanes typically have airfoil geometries designated by concave pressure sides and convex suction sides that extend axially between corresponding leading and trailing edges of the airfoils. Each airfoil is also typically disposed circumferentially between an outer arcuate shroud and an inner arcuate platform, thereby forming a nozzle segment. Multiple nozzle segments are interconnected to form the annular ring of the stationary turbine nozzle. Each nozzle segment may be cast to include one or more stator vanes disposed between the same outer arcuate shroud and inner arcuate platform. For example, a nozzle segment containing a single stator vane is typically referred to as a nozzle singlet, a nozzle segment containing two stator vanes is typically referred to as a nozzle doublet, nozzle segment containing three stator vanes is typically referred to as a nozzle triplet, and so on.

The components of the turbine stages (e.g., vanes and blades) are required to be able to withstand the thermal and oxidation conditions of the high temperature combustion gas during the course of operation. To protect turbine engine components from the extreme conditions, such components are typically coated with metallic bond coats that provide oxidation and/or corrosion resistance, and with ceramic thermal barrier coatings to provide thermal protection. However, many coating processes for forming bond coats and thermal barrier coatings require line-of-sight depositions. This poses problems when coating nozzle segments having multiple stator vanes because the inboard surfaces of the stator vanes are partially shadowed from the line-of-sight depositions. The resulting coatings typically have high variations in coating thicknesses due to the partial shadowing. Thus, there is an ongoing need for methods for coating nozzle segments having multiple stator vanes (e.g., nozzle doublets and triplets) to provide substantially uniform coatings with line-of sight coating techniques.

EP 0744529 discloses a method of applying a surface coating to nozzle segments of a turbine.

### SUMMARY

According to a first aspect the present invention a method for coating a nozzle segment having a plurality of stator vanes disposed between an outer shroud and an inner platform, the method comprising: separating the outer shroud and the inner platform along pathways that bisect a first stator vane and a second stator vane of the plurality of stator vanes; coating the first stator vane and the second stator vane using line-of-sight techniques after separating the outer shroud and the inner platform; rejoining the separated outer shroud after coating the first stator vane and the second stator vane; and rejoining the separated inner platform after coating the first stator vane and the second stator vane, wherein rejoining the separated outer shroud and rejoining the separated inner platform comprise performing a heat treatment process consisting of thermal diffusion bonding

According to a second aspect, the present invention provides a nozzle segment comprising: a first stator vane comprising a first pressure sidewall and a first suction sidewall, wherein the first pressure sidewall and the first suction sidewall each comprise a first coating formed using line-of-sight techniques and having a substantially uniform thickness; a second stator vane comprising a second pressure sidewall and a second suction sidewall, wherein the second pressure sidewall and the second suction sidewall each comprise a second coating formed using line-of-sight techniques and having a substantially uniform thickness; an outer shroud secured to the first stator vane and the second stator vane, the outer shroud having a first bond line disposed between the first stator vane and the second stator vane, and formed after the first coating and the second coating are formed; an inner platform secured to the first stator vane and the second stator vane at opposing ends from the outer shroud, the inner platform having a second bond line disposed between the first stator vane and the second stator vane, and formed after first coating and the second coating are formed, and wherein the first bond line and the second bond line are each formed with a heat treatment process comprising thermal bonding at a temperature ranging from about 1040°C to about 1200°C.

### BRIEF DESCRIPTION OF THE DRAWINGS

FIG. 1 is a flow diagram of a method for coating a nozzle segment having multiple stator vanes.
FIG. 2 is a top perspective view of a nozzle segment having multiple stator vanes disposed between an outer shroud and an inner platform.
FIG. 3 is a perspective view of the nozzle segment after separating the outer shroud and the inner platform.
FIG. 4 is a perspective view of the nozzle segment after rejoining the separated outer shroud and the separated inner platform.

### DETAILED DESCRIPTION

FIG. 1 is a flow diagram of method 10 for coating a nozzle segment having multiple stator vanes disposed between an outer shroud and an inner platform (e.g., nozzle doublets and triplets). As shown, method 10 includes steps 12-22, and initially involves identifying pathways along the outer shroud and the inner platform that bisect the stator vanes (step 12). The outer shroud and the inner platform are then separated along the identified pathways (steps 14 and 16) using a suitable separation technique (e.g., wire electrical discharge machining). The separation of the outer shroud and the inner platform splits the nozzle segment into multiple sub-segments, where each sub-segment desirably includes one of the multiple stator vanes. For example, in a nozzle doublet, the separation of the outer shroud and the inner platform splits the nozzle doublet into a pair of sub-segments, where each sub-segment includes a stator vane disposed between a portion of the outer shroud and a portion of the inner platform.

After the outer shroud and the inner platform are each separated, the stator vanes of the sub-segments are coated using a variety of coating techniques to form one or more coatings on the exposed surfaces of the stator vanes (step 18). Suitable coatings for the stator vanes include metallic protective coats (e.g., bond coats), thermal barrier coatings, and combinations thereof. As discussed below, the separation of the outer shroud and the inner platform allows the stator vanes to be placed apart from each other during the coating process, thereby allowing each stator vane to be coated with a line-of-sight coating technique. In one embodiment, this allows the resulting coatings to have substantially uniform thicknesses. As used herein with reference to a coating on a surface, the term "substantially uniform thickness" refers to coating thicknesses along the surface (e.g., along a surface of a stator vane) that remain within 10% of an average coating thickness for the given coating on the surface, disregarding thickness deviations due to topographical variations in the surface (e.g., cooling holes in the surface). Alternatively, in embodiments in which an non-uniform coating thickness is desirable (e.g., controlled changes in thickness), the separation of the outer shroud and the inner platform allow each stator vane to be coated with the desired changes in coating thicknesses.

After the coating process is complete, the outer shroud and the inner platform are each rejoined using a suitable joining process. The joining process forms bond lines between the sub-segments that are desirably capable of withstanding the extreme temperatures and pressures of the turbine stages of a gas turbine engine. The joining process also desirably preserves the integrities of the previously applied coatings (steps 20 and 22). The resulting nozzle segment, having the coated stator vanes, may then be reassembled with additional nozzle segments to form an annular ring of a stationary turbine nozzle. As discussed below, the separation and rejoining of the outer shroud and the inner platform allows the coatings formed on the stator vanes to have substantially uniformly thicknesses, thereby preserving the oxidation, corrosion, and/or thermal resistances of the stator vanes during the course of operation in a gas turbine engine.

FIGS. 2-4 are top perspective views of nozzle segment 24, which illustrate the use of method 10 (shown in FIG. 1) to form coatings on multiple stator vanes of nozzle segment 24. As shown in FIG. 2, nozzle segment 24 is a nozzle doublet that includes vanes 26 and 28, shroud 30, and platform 32. Vanes 26 are 28 are turbine-stage stator vanes secured between shroud 30 and platform 32. Vane 26 includes interior region 34, leading edge 36, trailing edge 38, pressure sidewall 40, and suction sidewall 42, where interior region 34 is a hollow interior portion of vane 26 that directs the flow of cooling air during operation. Pressure sidewall 40 is the concave pressure side of vane 26, which extends between leading edge 36 and trailing edge 38. Correspondingly, suction sidewall 42 is the convex suction side of vane 26, which also extends between leading edge 36 and trailing edge 38, and is the opposing surface to pressure sidewall 40.

Similarly, vane 28 includes interior region 44, leading edge 46, pressure sidewall 48, and suction sidewall 50, where interior region 44 is a hollow interior portion of vane 28 that directs the flow of cooling air during operation. Stator vane 28 also includes a trailing edge (not shown in FIG. 2) that corresponds to trailing edge 38 of stator vane 26. Pressure sidewall 48 is the concave pressure side of vane 28, which extends between leading edge 46 and the trailing edge of vane 28. Correspondingly, suction sidewall 50 is the convex suction side of vane 28, which also extends between leading edge 46 and the trailing edge of vane 28, and is the opposing surface to pressure sidewall 46.

Shroud 30 is an outer arcuate band secured to vanes 26 and 28, thereby allowing cooling air to enter interior regions 34 and 44 during operation. Shroud 30 includes leading edge 52, trailing edge 54, pressure side edge 56, and suction side edge 58, where leading edge 52 and trailing edge 54 are the upstream and downstream edges of shroud 30, respectively. Pressure side edge 56 and suction side edge 58 are the lateral edges of shroud 30, and are the edges that are secured to outer shrouds of adjacent nozzle segments (not shown) with leaf seal engagements to form a stationary turbine nozzle.

Correspondingly, platform 32 is an inner arcuate band secured to vanes 26 and 28, opposite of shroud 30. Platform 32 includes leading edge 60, trailing edge 62, pressure side edge 64, and suction side edge 66, where leading edge 60 and trailing edge 62 are the upstream and downstream edges of platform 32, respectively. Pressure side edge 64 and suction side edge 64 are the lateral edges of platform 32, and are the edges that are secured to inner platforms of adjacent nozzle segments (not shown) with leaf seal engagements to form the stationary turbine nozzle.

As shown, pressure sidewall 40 of vane 26 and suction sidewall 50 of vane 28 are outboard surfaces that are directly accessible with a line-of-sight coating technique. As a result, coatings may be readily deposited on pressure sidewall 40 and suction sidewall 50 with substantially uniform thicknesses. In contrast, however, suction sidewall 42 of vane 26 and pressure sidewall 48 of vane 28 are inboard surfaces, which partially shadow each other. The partial shadowing prevents line-of-sight coating techniques from evenly depositing coatings on suction sidewall 42 and pressure sidewall 48, thereby reducing coating thickness uniformity. The reduction in coating thickness uniformity correspondingly reduces the effectiveness of the formed coatings in providing corrosion, oxidation, and/or thermal resistance during the course of operation in a gas turbine engine.

As discussed above, method 10 is suitable for forming coatings on vanes 26 and 28, where the formed coatings have substantially uniform thicknesses on the outboard surfaces and the inboard surfaces. Prior to performing the coating process, pursuant to step 12 of method 10, pathways 68 and 70 are identified along shroud 30 and platform 32, respectively. Pathway 68 desirably extends from leading edge 52 to trailing edge 54 of shroud 30, between vanes 26 and 28. Similarly, pathway 70 desirably extends from leading edge 60 to trailing edge 62 of platform 32, also between vanes 26 and 28. As such, pathways 68 and 70 bisect vanes 26 and 28 along shroud 30 and shroud 32, respectively. While shown as linear pathways, pathways 68 and 70 may alternatively be non-linear pathways (e.g., curved lines and angled-segmented lines).

In one embodiment, pathways 68 and 70 are identified at locations along shroud 30 and platform 32 that are substantially even between vanes 26 and 28. This reduces the risk of damaging vanes 26 and 28 during the separation and rejoining steps of method 10. In an additional embodiment in which nozzle segment 24 includes existing bonds lines between vanes 26 and 28 (e.g., obtained during a previous manufacturing or restoration joining process), pathways 68 and 70 desirably follow the existing bond lines. This allows shroud 30 and platform 32 to be separated along the existing bond lines, which preserves the alloy microstructures of shroud 30 and platform 32.

After pathways 68 and 70 are identified, shroud 30 and platform 32 are separated along pathways 68 and 70, pursuant to steps 14 and 16 of method 10. Shroud 30 and platform 32 may be separated using a variety of techniques that are suitable for cutting the alloys of shroud 30 and platform 32 without damaging vanes 26 and 28. In one embodiment, shroud 30 and platform 32 are separated (simultaneously or sequentially) using wire electrical discharge machining (EDM). In this embodiment, nozzle segment 22 is placed in an aqueous bath, and a conductive wire is aligned with pathways 68 and 60 at leading edges 52 and 60, or at trailing edges 54 and 62. Electrical discharges are then sent through the conductive wire, thereby vaporizing successive portions of shroud 30 and platform 32 in the vicinity of the conductive wire. The wire is then passed along pathways 68 and 70 to separate nozzle segment 22 into separate sub-segments, thereby bisecting vanes 26 and 28.

FIG. 3 shows nozzle segment 24 (shown in FIG. 2) separated into sub-segments 24a and 24b, where sub-segment 24a includes vane 26 disposed between shroud portion 30a and platform portion 32a, and sub-segment 24b includes vane 28 disposed between shroud portion 30b and platform portion 32b. Shroud portions 30a and 30b are the separated portions of shroud 30 (shown in FIG. 2), and respectively include split edges 72 and 74 formed along pathway 68 (shown in FIG. 2) during the separation process of step 14 of method 10. Correspondingly, platform portions 32a and 32b are the separated portions of platform 32 (shown in FIG. 2), and respectively include split edges 76 and 78 formed along pathway 70 (shown in FIG. 2) during the separation process of step 16 of method 10. As further shown in FIG. 3, vane 28 includes trailing edge 80, which is the trailing edge of vane 28, as discussed above.

After the separation process, sub-segments 24a and 24b are placed apart from each other, and vanes 26 and 28 are coated to form one or more protective coatings, pursuant to step 18 of method 10. Prior to the coating process, one or more surfaces of shroud portions 30a and 30b and platform portions 32a and 32b may be masked to prevent the formation of coatings on the masked surfaces. Vanes 26 and 28 may then be coated using a variety of coating techniques, including line-of-sight coating techniques. For metallic bond and protective coatings, suitable coating techniques include electron-beam physical vapor deposition, low-pressure plasma spraying, cathodic arc deposition, vapor phase aluminide coating, pack cementation, chemical vapor deposition, electroplating, and combinations thereof.

For example, in an electron-beam physical vapor deposition process, sub-segments 24a and 24b are each placed on a rotatable mount in a vacuum chamber containing a target anode derived of the desired coating material. A charged tungsten filament then emits an electron beam that contacts the target anode, thereby ionizing the material of the target anode. The ionized particles then precipitate onto pressure sidewall 40 and suction side wall 42 of vane 26 and onto pressure sidewall 48 and suction side wall 50 of vane 28 to form the desired metallic coatings. Examples of suitable materials for the metallic coatings include aluminum, platinum, MCrAlY alloys, combinations thereof. Examples of suitable average thicknesses for the metallic coatings on vanes 26 and 28 range from about 25 micrometers to about 200 micrometers, with particularly suitable thicknesses ranging from about 50 micrometers to about 100 micrometers.

The above-discussed coating processes may also be used to form thermal barrier coatings on vanes 26 and 28. Suitable materials for the thermal barrier coatings include zirconia-based materials, where the zirconia is desirably modified with a stabilizer to prevent the formation of a monoclinic phase, and pyrochlores. Examples of suitable stabilizers include yttria, gadolinia, calcia, ceria, magnesia, and combinations thereof. Examples of suitable coating thicknesses for the thermal barrier coatings on stator vanes 26 and 28 range from about 25 micrometers to about 1,000 micrometers, with particularly suitable coating thicknesses ranging from about 100 micrometers to about 500 micrometers.

As discussed above, separating sub-segments 24a and 24b allows vanes 26 and 28 to be coated without interference from each other. Thus, when separated, pressure sidewall 40 and suction side wall 42 of vane 26, and pressure sidewall 48 and suction side wall 50 of vane 28, are each outboard surfaces that are directly accessible to the deposited coating materials. Thus, the coatings formed on pressure sidewalls 40 and 48, and on suction side walls 42 and 50, may have substantially uniform thicknesses. This preserves the corrosion, oxidation, and/or thermal resistance of the coatings during the course of operation in a gas turbine engine.

After the coating process is completed, sub-segments are placed together such split edges 72 and 74 of shroud portions 30a and 30b are substantially aligned, and such that split edges 76 and 78 of platform portions 32a and 32b are substantially aligned. Accordingly, during the rejoining process, split edges 72, 74, 76, and 78 function as faying surfaces. Pursuant to steps 20 and 22 of method 10, shroud portions 30a and 30b, and platform portions 32a and 32b are then each rejoined to reform shroud 30 and platform 32, respectively. As discussed above, the rejoining process forms bond lines (not shown in FIG. 3) between sub-segments 24a and 24b that are desirably capable of withstanding the extreme temperatures and pressures of the turbine stages of a gas turbine engine. Suitable techniques for the joining process may include any process that produces a metallurgical bond, such as gas tungsten arc welding, electron beam welding, laser welding, brazing, diffusion brazing, transient liquid phase bonding, and combinations thereof.

In one embodiment the rejoining process involves thermal diffusion bonding. In this embodiment, split edges 72 and 74 are compressed together and are subjected to elevated temperatures to interdiffuse the materials of shroud portions 30a and 30b, and split edges 76 and 78 are compressed together and are subjected to elevated temperatures to interdiffuse the materials of platform portions 32a and 32b. This may be performed by compressing sub-segments 24a and 24b together at split edges 72 and 74 and at split edges 76 and 78, and placing the compressed sub-segments 24a/24b in a vacuum oven for a suitable temperature and duration to interdiffuse the materials.

Suitable temperatures and durations for the thermal diffusion bonding include those that sufficiently bond shroud portions 30a and 30b, that sufficiently bond platform portions 32a and 32b, and that also substantially preserve the integrities of the coatings applied to vanes 26 and 28. Examples of suitable temperatures for the thermal diffusion bonding range from about 1040°C (about 1900°F) to about 1200°C (about 2200°F), with particularly suitable temperatures ranging from about 1090°C (about 2000°F) to about 1150°C (about 2100°F). Examples of suitable durations for the thermal diffusion bonding include durations up to about one hour, with particularly suitable durations ranging from about 10 minutes to about 30 minutes.

In an alternative embodiment, the rejoining process involves a transient liquid phase bonding. In this embodiment, layers of one or more brazing materials are placed between split edges 72 and 74, and between split edges 76 and 78, and sub-segments 24a and 24b are subjected to elevated temperatures. The elevated temperatures liquefy the brazing materials, thereby allowing the liquefied brazing materials to interdiffuse with the alloys of sub-segments 24a and 24b. Suitable temperatures and durations for the transient liquid phase bonding include those discussed above for the thermal diffusion bonding.

FIG. 4 shows sub-segments 24a and 24b rejoined at bond lines 82 and 84, thereby reforming nozzle segment 24 with coated vanes 26 and 28. Bond lines 82 and 84 are the locations of the interdiffused materials from the joining process, and generally follow pathways 68 and 70 (shown in FIG. 2), respectively. As discussed above, method 10 provides a suitable means for protecting vanes 26 and 28 with coatings having substantially uniform thicknesses, and is particularly suitable for use in combination with the restoration of used nozzle segments (e.g., nozzle segment 24). The resulting nozzle segment 24, having coated vanes 26 and 28, may then undergo one or more post-processing steps before being reassembled with additional nozzle segments to form an annular ring of a stationary turbine nozzle. The formed coatings may then protect vanes 26 and 28 from oxidation, corrosion, thermal attacks during the course of operation in a gas turbine engine.

Although the present invention has been described with reference to preferred embodiments, workers skilled in the art will recognize that changes may be made in form and detail without departing from the scope of the invention, which is defined by the claims and their equivalents.

## Claims

1. A method (10) for coating a nozzle segment having a plurality of stator vanes disposed between an outer shroud and an inner platform, the method comprising:
separating (14, 16) the outer shroud and the inner platform along pathways that bisect a first stator vane and a second stator vane of the plurality of stator vanes;
coating (18) the first stator vane and the second stator vane using line-of-sight techniques after separating the outer shroud and the inner platform;
rejoining (20) the separated outer shroud after coating the first stator vane and the second stator vane; and
rejoining (22) the separated inner platform after coating the first stator vane and the second stator vane,
**characterized in** rejoining (20) the separated outer shroud and rejoining the separated inner platform comprise performing a heat treatment process consisting of thermal diffusion bonding ,

2. The method of claim 1, wherein separating (14, 16) the outer shroud and the inner platform along the pathways comprises wire electrical discharge machining the outer shroud and the inner platform along the pathways.

3. The method of claim 1 or 2, wherein coating (18) the first stator vane and the second stator vane comprises performing an electron-beam physical vapor deposition process on the first stator vane and on the second stator vane.

4. The method of claim 1, 2 or 3, wherein the first stator vane (26) and the second stator vane (28) each comprise a pressure sidewall (40, 48) and a suction sidewall (42, 50), wherein after coating the first stator vane and the second stator vane, each of the pressure sidewalls and each of the suction sidewalls comprises a coating having a substantially uniform thickness.

5. The method of any one of claims 1 to 4, wherein the heat treatment process is performed at a temperature ranging from about 1040°C to about 1200°C.

6. The method of claim 5, wherein the temperature of the heat treatment process ranges from about 1090°C to about 1150°C.

7. The method of any preceding claim comprising:
identifying (12) a frst pathway along the outer shroud that bisects a first stator vane and a second stator vane of the plurality of stator vanes;
identifying (12) a second pathway along the inner platform that bisects the first stator vane and the second stator vane;
separating (14) the outer shroud along the identified first pathway to form a first shroud portion secured to the first stator vane and a second shroud portion secured to the second stator vane;
separating (16) the inner platform along the identified second pathway to form a first platform portion secured to the first stator vane and a second platform portion secured to the second stator vane;
forming (18) a first coating on the first stator vane after separating the outer shroud and the inner platform;
forming (18) a second coating on the second stator vane after separating the outer shroud and the inner platform;
rejoining (20) the first shroud portion and the second shroud portion; and
rejoining (22) the first platform portion and the second platform portion.

8. The method of claim 7, wherein separating (14) the outer shroud along the identified first pathway comprises wire electrical discharge machining the outer shroud along the identified first pathway.

9. The method of claim 7 or 8, wherein separating (16) the inner platform along the identified second pathway comprises wire electrical discharge machining the inner platform along the identified second pathway.

10. A nozzle segment (24) comprising:
a first stator vane (26) comprising a first pressure sidewall and a first suction sidewall, wherein the first pressure sidewall and the first suction sidewall each comprise a first coating formed using line-of-sight techniques and having a substantially uniform thickness;
a second stator vane (28) comprising a second pressure sidewall and a second suction sidewall, wherein the second pressure sidewall and the second suction sidewall each comprise a second coating formed using line-of-sight techniques and having a substantially uniform thickness;
an outer shroud (30) secured to the first stator vane and the second stator vane, the outer shroud having a first bond line disposed between the first stator vane and the second stator vane, and formed after the first coating and the second coating are formed;
an inner platform (32) secured to the first stator vane and the second stator vane at opposing ends from the outer shroud, the inner platform having a second bond line disposed between the first stator vane and the second stator vane, and formed after first coating and the second coating are formed,
**characterized in that** the first bond line and the second bond line are each formed with a heat treatment process comprising thermal bonding at a temperature ranging from about 1040°C to about 1200°C.

11. The nozzle segment of claim 10, wherein the first coating and the second coating are each formed from at least one material selected from the group consisting of aluminum, platinum, MCrAIY alloys, ceramic materials, and combinations thereof.

12. The nozzle segment of claim 10 or 11, wherein the first coating and the second coating each comprises an electron beam physical vapor deposition coating.

13. The nozzle segment of claim 10, 11 or 12, wherein the first coating and the second coating each have a coating thickness ranging from about 25 micrometers to about 1,000 micrometers, preferably from about 25 micrometers to about 200 micrometers.

## Patentansprüche

1. Verfahren (10) zum Beschichten eines Düsensegments mit einer Mehrzahl von Statorleitschaufeln, die zwischen einem äußeren Mantel und einer inneren Plattform angeordnet sind, wobei das Verfahren Folgendes beinhaltet:
Trennen (14, 16) des äußeren Mantels und der inneren Plattform entlang von Wegen, die eine erste Statorleitschaufel und eine zweite Statorleitschaufel der Mehrzahl von Statorleitschaufeln halbieren;
Beschichten (18) der ersten Statorleitschaufel und der zweiten Statorleitschaufel unter Verwendung von Sichtlinientechniken nach dem Trennen des äußeren Mantels und der inneren Plattform;
Wiederverbinden (20) des getrennten äußeren Mantels nach dem Beschichten der ersten Statorleitschaufel und der zweiten Statorleitschaufel; und
Wiederverbinden (22) der getrennten inneren Plattform nach dem Beschichten der ersten Statorleitschaufel und der zweiten Statorleitschaufel,
**dadurch gekennzeichnet,**
**dass** das Wiederverbinden (20) des getrennten äußeren Mantels und das Wiederverbinden (22) der getrennten inneren Plattform das Ausführen eines Wärmebehandlungsprozesses beinhaltet, der aus thermischem Diffusionsbonden besteht.

2. Verfahren nach Anspruch 1,
wobei das Trennen (14, 16) des äußeren Mantels und der inneren Plattform entlang der Wege eine Drahterosionsbearbeitung des äußeren Mantels und der inneren Plattform entlang der Wege beinhaltet.

3. Verfahren nach Anspruch 1 oder 2,
wobei das Beschichten (18) der ersten Statorleitschaufel und der zweiten Statorleitschaufel das Durchführen einer physikalischen Elektronenstrahl-Gasphasenabscheidung an der ersten Statorleitschaufel und an der zweiten Statorleitschaufel beinhaltet.

4. Verfahren nach Anspruch 1, 2 oder 3,
wobei die erste Statorleitschaufel (26) und die zweite Statorleitschaufel (28) jeweils eine Druckseitenwand (40, 48) und eine Sogseitenwand (42, 50) aufweisen, wobei nach dem Beschichten der ersten Statorleitschaufel und der zweiten Statorleitschaufel die Druckseitenwände und die Sogseitenwände jeweils eine Beschichtung mit einer im wesentlichen gleichmäßigen Dicke aufweisen.

5. Verfahren nach Anspruch 1 bis 4,
wobei der Wärmebehandlungsprozess bei einer Temperatur im Bereich von etwa 1040°C bis etwa 1200°C ausgeführt wird.

6. Verfahren nach Anspruch 5
wobei die Temperatur des Wärmebehandlungsprozesses im Bereich von etwa 1090°C bis etwa 1150°C liegt.

7. Verfahren nach einem der vorhergehenden Ansprüche, aufweisend:
Identifizieren (12) eines ersten Wegs entlang des äußeren Mantels, der eine erste Statorleitschaufel und eine zweite Statorleitschaufel der Mehrzahl von Statorleitschaufeln halbiert;
Identifizieren (12) eines zweiten Wegs entlang der inneren Plattform, der die erste Statorleitschaufel und die zweite Statorleitschaufel halbiert;
Trennen (14) des äußeren Mantels entlang des identifizierten ersten Wegs, um einen an der ersten Statorleitschaufel befestigten ersten Mantelbereich und einen an der zweiten Statorleitschaufel befestigten zweiten Mantelbereich zu bilden;
Trennen (16) der inneren Plattform entlang des identifizierten zweiten Wegs, um einen an der ersten Statorleitschaufel befestigten ersten Plattformbereich und einen an der zweiten Statorleitschaufel befestigten zweiten Plattformbereich zu bilden;
Bilden (18) einer ersten Beschichtung auf der ersten Statorleitschaufel nach dem Trennen des äußeren Mantels und der inneren Plattform;
Bilden (18) einer zweiter Beschichtung auf der zweiten Statorleitschaufel nach dem Trennen des äußeren Mantels und der inneren Plattform;
Wiederverbinden (20) des ersten Mantelbereichs und des zweiten Mantelbereichs; und
Wiederverbinden (22) des ersten Plattformbereichs und des zweiten Plattformbereichs.

8. Verfahren nach Anspruch 7,
wobei das Trennen (14) des äußeren Mantels entlang des identifizierten ersten Wegs eine Drahterosionsbearbeitung des äußeren Mantels entlang des identifizierten ersten Wegs beinhaltet.

9. Verfahren nach Anspruch 7 oder 8,
wobei das Trennen (16) der inneren Plattform entlang des identifizierten zweiten Wegs eine Drahterosionsbearbeitung der inneren Plattform entlang des identifizierten zweiten Wegs beinhaltet.

10. Düsensegment (24), aufweisend:
eine erste Statorleitschaufel (26), die eine erste Druckseitenwand und eine erste Sogseitenwand aufweist, wobei die erste Druckseitenwand und der erste Sogseitenwand jeweils eine erste Beschichtung aufweisen, die unter Verwendung von Sichtlinientechniken gebildet ist und eine im Wesentlichen gleichmäßige Dicke aufweist;
eine zweite Statorleitschaufel (28), die eine zweite Druckseitenwand und eine zweite Sogseitenwand aufweist, wobei die zweite Druckseitenwand und die zweite Sogseitenwand jeweils eine zweite Beschichtung aufweisen, die unter Verwendung von Sichtlinientechniken gebildet ist und eine im Wesentlichen gleichmäßige Dicke aufweist;
einen äußeren Mantel (30), der an der ersten Statorleitschaufel und der zweiten Statorleitschaufel befestigt ist, wobei der äußere Mantel eine erste Verbindungslinie aufweist, die zwischen der ersten Statorleitschaufel und der zweiten Statorleitschaufel angeordnet ist und nach dem Bilden der ersten Beschichtung und der zweiten Beschichtung gebildet ist;
eine innere Plattform (32), die an der ersten Statorleitschaufel und der zweiten Statorleitschaufel an gegenüberliegenden Enden von dem äußeren Mantel befestigt ist, wobei die innere Plattform eine zweite Verbindungslinie aufweist, die zwischen der ersten Statorleitschaufel und der zweiten Statorleitschaufel angeordnet ist und nach dem Bilden der ersten Beschichtung und der zweiten Beschichtung gebildet ist, und **dadurch gekennzeichnet, dass** die erste Verbindungslinie und die zweite Verbindungslinie jeweils mittels eines Wärmebehandlungsprozesses gebildet sind, der eine thermische Verbindung bei einer Temperatur in einem Bereich von etwa 1040°C bis etwa 1200°C beinhaltet.

11. Düsensegment nach Anspruch 10,
wobei die erste Beschichtung und die zweite Beschichtung jeweils aus mindestens einem Material gebildet sind, das aus der Gruppe bestehend aus Aluminium, Platin, MCrAIY-Legierungen, Keramikmaterialien und Kombinationen davon ausgewählt ist.

12. Düsensegment nach Anspruch 10 oder 11,
wobei die erste Beschichtung und die zweite Beschichtung jeweils eine durch physikalische Elektronenstrahl-Gasphasenabscheidung gebildete Beschichtung beinhalten.

13. Düsensegment nach Anspruch 10, 11 oder 12,
wobei die erste Beschichtung und die zweite Beschichtung jeweils eine Beschichtungsdicke im Bereich von etwa 25 Mikrometer bis etwa 1000 Mikrometer, vorzugsweise von etwa 25 Mikrometer bis etwa 200 Mikrometer, aufweisen.

## Revendications

1. Une méthode (10) pour appliquer un revêtement à un segment de buse ayant une pluralité d'aubes de stator disposées entre une gaine extérieure et une plate-forme intérieure, la méthode comprenant :
la séparation (14, 16) de la gaine extérieure et de la plate-forme intérieure le long de chemins qui coupent une première aube de stator et une deuxième aube de stator de la pluralité d'aubes de stator ;
l'application d'un revêtement (18) à la première aube de stator et à la deuxième aube de stator en utilisant des techniques de ligne de visée après avoir séparé la gaine extérieure et la plate-forme intérieure ;
la réunion (20) de la gaine extérieure séparée après avoir appliqué le revêtement à la première aube de stator et à la deuxième aube de stator ; et
la réunion (22) de la plate-forme intérieure séparée après avoir appliqué le revêtement à la première aube de stator et à la deuxième aube de stator,
**caractérisée en ce que** la réunion (20) de la gaine extérieure séparée et la réunion de la plate-forme intérieure séparée comprennent l'exécution d'un procédé de traitement par la chaleur consistant en un soudage par diffusion thermique.

2. La méthode de la revendication 1, dans laquelle la séparation (14, 16) de la gaine extérieure et de la plate-forme intérieure le long des chemins comprend l'usinage par électro-érosion par fil de la gaine extérieure et de la plate-forme intérieure le long des chemins.

3. La méthode des revendications 1 ou 2, dans laquelle l'application d'un revêtement (18) à la première aube de stator et à la deuxième aube de stator comprend l'utilisation d'un procédé de dépôt physique en phase vapeur par un faisceau d'électrons sur la première aube de stator et sur la deuxième aube de stator.

4. La méthode de la revendication 1, 2 ou 3, dans laquelle la première aube de stator (26) et la deuxième aube de stator (28) comprennent chacune une paroi latérale de pression (40, 48) et une paroi latérale d'aspiration (42, 50), dans laquelle après avoir appliqué le revêtement à la première aube de stator et à la deuxième aube de stator, chacune des parois latérales de pression et chacune des parois latérales d'aspiration comprend un revêtement ayant une épaisseur sensiblement uniforme.

5. La méthode d'une quelconque des revendications 1 à 4, dans laquelle le procédé de traitement par la chaleur est exécuté à une température s'étendant de 1040 °C environ à 1200 °C environ.

6. La méthode de la revendication 5, dans laquelle la température du procédé de traitement par la chaleur s'étend de 1090 °C environ à 1150 °C environ.

7. La méthode de n'importe quelle revendication précédente comprenant :
l'identification (12) d'un premier chemin le long de la gaine extérieure qui coupe une première aube de stator et une deuxième aube de stator de la pluralité d'aubes de stator ;
l'identification (12) d'un deuxième chemin le long de la plate-forme intérieure qui coupe la première aube de stator et la deuxième aube de stator ;
la séparation (14) de la gaine extérieure le long du premier chemin identifié de manière à former une première partie de gaine fixée à la première aube de stator, et une deuxième partie de gaine fixée à la deuxième aube de stator ;
la séparation (16) de la plate-forme intérieure le long du deuxième chemin identifié de manière à former une première partie de plate-forme fixée à la première aube de stator, et une deuxième partie de plate-forme fixée à la deuxième aube de stator ;
la formation (18) d'un premier revêtement sur la première aube de stator après avoir séparé la gaine extérieure et la plate-forme intérieure ;
la formation (18) d'un deuxième revêtement sur la deuxième aube de stator après avoir séparé la gaine extérieure et la plate-forme intérieure ;
la réunion (20) de la première partie de gaine et de la deuxième partie de gaine ; et
la réunion (22) de la première partie de plate-forme et de la deuxième partie de plate-forme.

8. La méthode de la revendication 7, dans laquelle la séparation (14) de la gaine extérieure le long du premier chemin identifié comprend l'usinage par électro-érosion par fil de la gaine extérieure le long du premier chemin identifié,

9. La méthode de la revendication 7 ou 8, dans laquelle la séparation (16) de la plate-forme intérieure le long du deuxième chemin identifié comprend l'usinage par électro-érosion par fil de la plate-forme intérieure le long du deuxième chemin identifié,

10. Un segment de buse (24) comprenant :
une première aube de stator (26) comprenant une première paroi latérale de pression et une première paroi latérale d'aspiration, dans laquelle la première paroi latérale de pression et la première paroi latérale d'aspiration comprennent chacune un premier revêtement formé en utilisant des techniques de ligne de visée et ayant une épaisseur substantiellement uniforme ;
une deuxième aube de stator (28) comprenant une deuxième paroi latérale de pression et une deuxième paroi latérale d'aspiration, dans laquelle la deuxième paroi latérale de pression et la deuxième paroi latérale d'aspiration comprennent chacune un deuxième revêtement formé en utilisant des techniques de ligne de visée et ayant une épaisseur sensiblement uniforme ;
une gaine extérieure (30) fixée à la première aube de stator et à la deuxième aube de stator, la gaine extérieure ayant une première ligne de soudure située entre la première aube de stator et la deuxième aube de stator, et formée après que le premier revêtement et le deuxième revêtement aient été formés ;
et une plate-forme intérieure (32) fixée à la première aube de stator et à la deuxième aube de stator à des extrémités opposées par rapport à la gaine extérieure, la plate-forme intérieure ayant une deuxième ligne de soudure située entre la première aube de stator et la deuxième aube de stator, et formée après que le premier revêtement et le deuxième revêtement aient été formés, et
**caractérisée en ce que** la première ligne de soudure et la deuxième ligne de soudure sont chacune formée par un procédé de traitement par la chaleur comprenant un soudage thermique à une température s'étendant de 1040 °C environ à 1200 °C environ.

11. Le segment de buse de la revendication 10, dans laquelle le premier revêtement et le deuxième revêtement sont chacun formé à partir d'au moins un matériau sélectionné dans le groupe constitué de l'aluminium, du platine, des alliages de MCrAIY, des matériaux céramiques, et des combinaisons de ceux-ci.

12. Le segment de buse de la revendication 10 ou 11, dans laquelle le premier revêtement et le deuxième revêtement comprennent chacun un revêtement appliqué par dépôt physique en phase vapeur par un faisceau d'électrons,

13. Le segment de buse de la revendication 10, 11 ou 12, dans laquelle le premier revêtement et le deuxième revêtement ont chacun une épaisseur de revêtement s'étendant d'environ 25 micromètres à environ 1000 micromètres, et de préférence d'environ 25 micromètres à environ 200 micromètres.
